

Oct. 28, 1969

M. D. ZEISBERG

3,474,616

PRODUCT AND PROCESS

Filed June 29, 1967

FIG. 1



FIG. 3



FIG. 2



FIG. 5



FIG. 4



FIG. 6



INVENTOR  
MILLARD D. ZEISBERG

BY

*Millard D. Zeisberg*

ATTORNEY

1

3,474,616

## PRODUCT AND PROCESS

Millard David Zeisberg, Newark, Del., assignor to E. I. du Pont de Nemours and Company, Wilmington, Del., a corporation of Delaware

Filed June 29, 1967, Ser. No. 649,944

Int. Cl. D02g 3/36; D01d 11/06; B44d 1/22

U.S. Cl. 57—164

7 Claims

### ABSTRACT OF THE DISCLOSURE

Plexifilamentary strand material is impregnated uniformly with particulate material. A rod-shaped batt of longitudinally collapsed plexifilamentary strand material is mounted so that a cone of the strand material pulled from one end of the batt is at least partially submerged in a suspension of the particulate material. The strand material is pulled continuously from the end of the batt through the suspension.

### Background

This invention relates to the impregnation of continuous plexifilamentary strands with particulate materials and to the composite structures so prepared.

Numerous products are known which combine particulate materials with continuous strands of tow, yarn, or roving. These include, for example: sized textile yarns, such as cotton strands sized with starch; electrical conductors formed by impregnating or coating rayon fibers with graphite or conductive carbon; strands comprising short-fiber asbestos formed from dispersions of the short fibers with a variety of additives (see, for example, Wilke et al. U.S. Patent No. 2,972,221); further strands comprising short-fiber asbestos combined with longer strands of cotton, rayon, or nylon or with continuous metallic wires; fiber-reinforced strands combining fibrous material with cementitious materials (see British patent specification 1,042,606); strands produced directly from slurries of wood pulp and then woven into sheets or wrapped around wires for insulation; and any number of composite structures resulting from drawing strands through mixtures of particulate solids with binders to coat and/or impregnate the strands.

When a flexible strand or roving is to be combined with other materials, it has been necessary to employ low viscosity solutions or dispersions in order to promote penetration of impregnant to the core of the strand. Viscous agents or large-particle suspensions invariably coat or encase the strands rather than uniformly impregnate the strand material. The formation of composite flexible strands using non-fibrous particles, i.e., particles of globular, spherical, flake, or plate-like shape, has been difficult and ordinarily produces composite strands in which the continuous fibrous material and/or added binder constitute a large proportion by weight.

Certain particulate materials have been intractable because of size, shape, or intrinsic nature, and frequently no feasible or economical method is available to form strands of these particles in a supporting matrix to provide the desired characteristics. Often the very presence of a binder, or the large quantity of binder required to hold the particulate materials together, interferes with obtaining desired physical characteristics, e.g., flexibility, conformability, porosity, and absorptivity.

2

Belgian Patent No. 670,293, granted Oct. 15, 1965, discloses a method for preparing a rod-shaped batt of longitudinally collapsed continuous plexifilamentary strand material. A plexifilamentary strand is a yarn-like strand comprising a three-dimensional integral plexus of synthetic organic polymeric, fibrous elements having the structural configuration of film-fibrils which exhibit a thickness of less than about 4 microns and which are so finely divided as to impart to the strand a total surface area of at least 2 m<sup>2</sup>/gm. Preferred plexifilamentary strands are those disclosed in Blades and White U.S. Patent No. 3,081,519, issued Mar. 19, 1963.

The rod-shaped batt disclosed in the Belgian patent is characterized in that, from either end, or from new ends formed by breaking the batt at any point along its length, a single continuous plexifilamentary strand can readily be pulled. The strand comes off the batt as an integral, generally circular, open network which collapses radially to a yarn-like strand at a point downstream. Thus, the strand assumes a cone-shaped configuration as it is pulled from the end of the batt, with the apex of the cone pointed in the direction of strand travel.

### Summary of the invention

According to this invention there is provided a composite structure comprising solid particulate material uniformly distributed throughout a plexifilamentary strand. The invention also provides a method for producing such a structure which comprises the steps of (1) providing a suspension of solid particulate material in a dispersing medium, (2) mounting a rod-shaped batt of longitudinally collapsed continuous plexifilamentary strand material such that a cone of plexifilamentary strand material pulled from one end of said batt is at least partially immersed in said suspension, and (3) continuously pulling said plexifilamentary strand from said batt through said suspension.

### Brief description of the drawings

FIGURE 1 is a partly sectional drawing illustrating one embodiment of this invention wherein a rod-shaped plexifilamentary batt is immersed in a suspension of particulate material and an end of plexifilamentary strand is continuously withdrawn while at least a portion of its cone remains submerged.

FIGURE 2 is a representation of a plexifilamentary batt suitable for use according to this invention.

FIGURE 3 is an enlarged view along the opened length of a plexifilamentary strand impregnated throughout with particulate material.

FIGURE 4 illustrates in partial cross-section an alternative method for impregnation according to this invention wherein the batt is mounted outside of the suspension of particulate material.

FIGURE 5 is analogous to FIGURE 3, showing preferential alignment of acicular particles generally parallel to the longitudinal axis of the plexifilamentary strand.

FIGURE 6 is a schematic drawing of an over-all equipment arrangement permitting continuous coupled operation according to this invention.

### Description of the preferred embodiments

With reference now to FIGURE 2, a suitable plexifilamentary batt 1 is discussed in more detail. The cross-sectional shape of batt 1 is circular, but oval, polygonal, and other cross-sectional shapes are equally suitable. These

cross-sectional shapes can be solid or hollow, the latter resulting either if the plexifilament is collected in an annular space or if the solid batt is later hollowed by axial boring. A single continuous plexifilamentary strand 2 can be withdrawn from either end of batt 1. A batt 1, or any section broken from it, ordinarily has a convex end 5 and a concave end 4, convex end 5 being the one first formed and concave end 4 the one from which continuous plexifilamentary strand 2 is preferably withdrawn. In collecting a plexifilamentary strand in the form of batt 1, the strand balloons so that the multitudinous interconnected film-fibril elements constituting the strand at any point are deposited throughout an enlarged generally circular area, which area should be at least one-fourth and preferably at least two-thirds of the area of concave end 4 of batt 1. Subsequent pulling of the plexifilamentary strand 2 from an end of batt 1 generates a generally conical section 3 of plexifilament, cone 3 having an apex away from the end of batt 1 along the withdrawal direction and a base at the end of batt 1 corresponding to the generally circular area of previous deposition. Plexifilamentary strands with deniers from 15 to 100,000 or greater can be collected as batts and subsequently pulled from them. The batt 1 ordinarily has a length of from  $\frac{1}{25}$  to  $\frac{1}{500}$ , preferably  $\frac{1}{400}$  to  $\frac{1}{200}$ , of the length of plexifilamentary strand 2 which can be pulled from it; and the density of suitable batts 1 is generally between about 16 and 240 kg./m.<sup>3</sup>, preferably between about 110 and 135 kg./m.<sup>3</sup>.

One embodiment of the process of this invention is now discussed with reference to FIGURE 1. A suspension of particulate material 8 in dispersing medium 6 is provided in a suitable container 12. A plexifilamentary batt 1 is submerged in the suspension, and a continuous plexifilamentary strand 2 is continuously pulled from end 4 of batt 1 through and away from the suspension. As discussed hereinabove, withdrawing the strand 2 creates a cone 3 of plexifilamentary material, and it is critical to this improved strand-impregnation process that at least a portion of cone 3 be immersed below the upper level 7 of the suspension. As indicated in FIGURE 1, particulate material 8 is withdrawn substantially uniformly dispersed within strand 2.

FIGURE 3 is an enlarged representation of an impregnated plexifilamentary strand 2, the strand having been opened by lateral tensioning to render it substantially planar and to reveal the internal distribution of particles 8. The fineness of the multitudinous interconnected film-fibrils 9 forming the plexus of strand 2 results in so extensive contact with the particles 8 that the composite structure is unexpectedly coherent and durable without the use of binders. For example, a dry composite strand containing 20 parts by weight of wood flour per part of linear polyethylene film-fibrils loses as little as 6% by weight of the wood flour after a one-foot (30.5 cm.) long strand is vigorously shaken twice.

Another embodiment of the process of this invention is depicted schematically in FIGURE 4. A suitable container 12 is provided with a suspension of particulate material 8 in a dispersing medium 6. Batt 1 is mounted generally outside the suspension so that, when plexifilamentary strand 2 is pulled downward from its face 4, cone 3 is at least partially immersed below level 7 of the suspension. A guide roll or rod 17 within the suspension translates the force of strand removal into a downward force at face 4 of batt 1. As in FIGURE 1, strand 2 leaves the suspension with particles 8 intimately distributed throughout. The amount of particles thus incorporated generally increases as more of cone 3 is immersed, and maximum impregnation results when the level of suspension is raised to that shown by dotted line 10 corresponding to immersion of face 4 of batt 1.

FIGURE 6 represents schematically an overall coupled process for preparing a finished strand, any or all of the auxiliary functions of which may be used as desired. If twist is to be imparted to the final strand, it is convenient-

ly obtained by mounting batt 1 in a holder 16 which can rotate as indicated by arrow 19. In order to maintain level 7 of the suspension and to replenish particulate material 8 removed with strand 2, means for continuously introducing fresh suspension are required, such as indicated by side-tube 18. Ordinarily the concentration of particles 8 in fresh suspension is greater than that maintained in vessel 12. By providing, for instance, a set of friction-rolls 20 and a set of draw-rolls 22, stretch-elongation is imparted to strand 2 in the region 21 therebetween. A drying region 24, for instance an over 23 supplied with heated gases at 25, may also be provided. Finally, the finished strand is either wound-up into a suitable package 26 or drawn on to other alternative processing steps.

Particulate material useful in this invention can be substantially any finely divided (i.e., volume less than about 1 cubic millimeter), dispersible solids with any particle shape, e.g., spherical, globular, flake, plate-like, acicular, or fibrous. Examples of suitable particulate materials include wood flour, asbestos shorts, potassium titanate, diatomaceous earth, nylon flock, lead powder, aluminum flake, acicular boron nitride, activated charcoal, conductive carbon, and the like. Suitable suspensions can be mechanically maintained or colloidally dispersed or a suspending agent can be used.

Liquid dispersing mediums are ordinarily employed. Water is the most common dispersing medium, but many other liquids, such as alkanols and halogenated alkanes, form suitable suspensions, as are well-known in the art. The dispersing medium can also be gaseous, e.g., fluidized beds of the particulate materials. As is readily apparent, numerous other additives can be dissolved or suspended in the dispersing medium, these additives including, for example, wetting agents, binders, dyes, buffering agents, and the like.

The film-fibrils constituting a plexifilamentary strand have a predominantly longitudinal orientation, as is evidenced by much greater resistance to tearing by longitudinally than by transversely applied forces. The introduction of acicular particles according to the process of this invention also results in their being predominantly longitudinally oriented, which effect is enhanced by subsequently drawing the impregnated strand. FIGURE 5 shows the longitudinal orientation of acicular particles 11 in a strand 2 laterally opened as in FIGURE 3.

The following examples are representative of the breadth of application of this invention. In them, all ratios and percentages are by weight unless specifically indicated otherwise. The batt used in most of the examples is a 4.84 cm. diameter batt of plexifilamentary linear polyethylene as described in Example I of the aforesaid Belgian Patent No. 670,293. Differing sizes, shapes, and polymeric compositions of batt are indicated where applicable, this particular one being designated simply as "a 4.84 cm. diameter polyethylene batt." While linear polyethylene is the preferred polymer, any polymer which can form plexifilaments and which can be collected as a batt according to Belgian Patent No. 670,293 is suitable.

#### EXAMPLE I

A 4.84 cm. diameter polyethylene batt is impregnated with minus 300 mesh wood flour (Eastern White Pine or Douglas Fir) by the process of this invention. Except for the lack of continuous drying, the apparatus and procedure employed are as shown in FIGURE 6. The suspension employed is composed of 2.55 gm. of wood flour, 100 cc. of water containing 1% of isoctyl phenyl polyethoxy ethanol wetting agent, and 3.14 gm. (based on solids) of aqueous dispersion of ethyl acrylate polymer particles of less than 0.5 micron size. The batt is mounted in the holder but is not rotated. With its cone immersed in the suspension, the polyethylene plexifilament is withdrawn at about 6.8 meters/min. and is drawn (region 21 of FIGURE 6) 13.5%. The resulting strand is cut into suc-

cessive 1.27 meter lengths and dried. Approximate impregnation equilibrium is reached after about 20 samples are obtained, characterization of samples 27, 29, 31 and 33 being given in Table I.

TABLE I.—CHARACTERIZATION OF WOOD-FLOUR IMPREGNATED STRANDS

| Sample No. | Denier | Strand Diameter (mm.) | Breaking Strength (kg.) | Residual Elongation Percent |
|------------|--------|-----------------------|-------------------------|-----------------------------|
| 27-----    | 4,566  | 0.87                  | 2.01                    | 36.6                        |
| 29-----    | 5,141  | 0.92                  | 1.92                    | 36.7                        |
| 31-----    | 5,285  | 0.98                  | 2.06                    | 39.0                        |
| 33-----    | 5,211  | 0.90                  | 2.11                    | 39.6                        |

Due to the presence of acrylic binder, the bulky strand is free of dusting. The weight of dry wood flour retained is between 6.5 and 7.5 times the weight of the original plexifilamentary strand. The strands are useful as filler cords for conductive cables.

## EXAMPLE II

A 4.84 cm. diameter polyethylene batt is used for preparing a strand impregnated with medium length asbestos fiber. Apparatus and procedure are in accordance with FIGURE 6. The asbestos "shorts" (predominantly crocidolite) exhibit the following size distribution in a "RO-Tap" 30-minute, 100-gm. analysis:

| Screen size, mesh: | Retained weight, gm. |
|--------------------|----------------------|
| 6 -----            | 0                    |
| 14 -----           | 4.50                 |
| 20 -----           | 30.25                |
| 28 -----           | 21.75                |
| 35 -----           | 18.75                |
| 65 -----           | 11.00                |

A suspension is prepared from 200 gm. of these asbestos shorts, 30 cc. of a sodium silicate solution, and 40 cc. of non-ionic isoctyl phenyl polyethoxy ethanol in 8 liters of water. The water-solution of sodium silicate has a specific gravity at 60° F. (15.5° C.) of 50.25° Bé. and contains 28.50% SiO<sub>2</sub> and 15.00% Na<sub>2</sub>O.

Polyethylene plexifilamentary strand is withdrawn from the batt through the suspension at 12.5 meters/min. while the batt is rotated at 550 r.p.m. Subsequently the impregnated strand is drawn 17.5% and dried. A 2.54 meter long sample is taken for every 7.5 to 10.0 meter length of dried strand, with results shown in Table II.

TABLE II.—CHARACTERIZATION OF ASBESTOS-FIBER IMPREGNATED STRANDS

| Sample No. | Dry Weight (gm./10 meters) | Percent Polyethylene | Asbestos Cut |
|------------|----------------------------|----------------------|--------------|
| 3-----     | 5.63                       | 13.0                 | 8.8          |
| 4-----     | 5.70                       | 12.9                 | 8.7          |
| 5-----     | 4.87                       | 15.1                 | 10.2         |
| 6-----     | 7.00                       | 10.6                 | 7.1          |
| 7-----     | 7.20                       | 10.3                 | 6.9          |

Asbestos cut is the approximate number of 100 yard (91.44 meter) lengths required to weigh one pound (0.454 kg.). Asbestos yarns containing at least 85%, but less than 90%, asbestos are labeled "Grade A" in the industry. The composite strands can be woven to provide thick, decorative, high drape fabrics for use as drapery, wall hangings, and the like.

## EXAMPLE III

A fabric woven from wood-flour impregnated polyethylene plexifilament is described.

The suspension employed for impregnation is composed of 300 gm. of the wood flour of Example I, 100

cc. of a resin emulsion, 8 liters of water, and 40 cc. of nonionic isoctyl phenyl polyethoxy ethanol wetting agent. The resin emulsion (Velsicol Chemical Corp. "Stikvel" P-65, said to be a cyclopentadiene derivative) is a tacky, non-drying, non-oxidizing emulsion containing 65% of solids which are less than 1 micron in diameter.

Impregnation is according to FIGURE 6. The 4.84 cm. diameter polyethylene batt is rotated at 1000 r.p.m.; strand is withdrawn at 27.5 meters/min.; a 22% stretch is imposed; and the impregnated strand is dried. It is characterized as follows:

Average weight—2.52 gm./10 meters  
Breaking strength—1.14 kg.

Residual Elongation—26.7%

A portion of the strand is woven into a conventional plain-weave fabric with 4.73 warp-yarns and 6.50 fill-yarns per centimeter. The 1.42 mm. thick fabric weighs 276 gm./m.<sup>2</sup>. It is smooth in appearance and is remarkably drapeable and soft for this thickness making it a highly desirable yet inexpensive fabric for decorative use such as in drapery and tapestry. Specific gravity of the fabric is only about 0.2.

## EXAMPLE IV

A suspension of fine acicular potassium titanate particles is formed by intensively mixing 30 gm. of the particles in 500 cc. of water. The volume is increased to 1350 cc. with water, and 150 cc. of 10% isoctyl phenyl polyethoxy ethanol wetting agent is added.

A 4.84 cm. diameter polyethylene batt is immersed in the suspension as shown in FIGURE 1, and impregnated strand is withdrawn without twisting at about 20 meters/min. Samples 1.27 meters long are taken throughout the run and dried. Results are shown in Table III.

TABLE III.—POTASSIUM TITANATE IMPREGNATED POLY-ETHYLENE STRANDS

| Sample No. | Dry Weight (gm./10 m.) | Percent Polyethylene |
|------------|------------------------|----------------------|
| 1-3-----   | 5.12-5.52              | 15.6-16.0            |
| 4-----     | 4.45                   | 19.8                 |
| 5-----     | 3.84                   | 22.3                 |
| 6-----     | 3.72                   | 23.4                 |
| 7-----     | 3.74                   | 23.1                 |
| 8-----     | 3.67                   | 23.0                 |
| 9-----     | 3.56                   | 24.4                 |
| 10-----    | 3.44                   | 25.2                 |
| 11-----    | 3.31                   | 26.0                 |
| 12-----    | 3.24                   | 26.0                 |
| 13-----    | 3.19                   | 27.5                 |

The suspension is not replenished during this operation. From the almost linear decrease in strand weight with time (sample number), at least after the fourth sample is taken, it is apparent that solids level in the remaining suspension is decreasing and that the plexus of strand material passing through the suspension preferentially concentrates the acicular particles within it.

## EXAMPLE V

A filter-cartridge prepared from impregnated strands of this invention is described. A 4.84 cm. diameter polyethylene batt is processed as shown in FIGURE 6 with zero twist. Strand is withdrawn at 25.5 meters/min., stretched 17%, and oven-dried to constant weight at below 120° C. (about 13° C. below the melting point of the linear polyethylene). The suspension employed is composed of 1200 gm. of a filter aid, 8 liters of water, and 200 cc. of 10% isoctyl phenyl polyethoxy ethanol wetting agent. The filter aid is finely divided diatomaceous earth of which 92% has particle sizes less than 40 microns, 79% less than 20 microns, 46% less than 10 microns, and none less than 2 microns. The ratio of wet to dry strand weights is about 4.35; and representative 50

cm. lengths of dry strand weigh from 10 to 11 gm./10 m. after processing into filter cartridges.

To produce the cartridge filter, the dried strand is first transferred from its collection spool onto a 5.08 cm. diaemter cardboard tube and then pulled over the end onto 25.4 cm. of the length of a 30 cm. long, 2.54 cm. diameter perforated core. The windup pattern used is known as an 8-traverse pattern in which 8 separate diamond crossover points progress around the outer circumference in a plane at right angles to the long axis of the perforated core. Final diameter of the completed cartridge is 4.25 cm.

The cartridge filter exhibits a pressure drop of 20.8 cm. of mercury for air flow through it of 84 liters/min. Filtration efficiency is tested using an aqueous suspension of carbon black of a particle size characterized as 0% greater than 18 microns, 25% greater than 10 microns, and 50% greater than 5 microns. Solids at a concentration of 15-20 parts per million are fed to the filter at 2.3 grams per hour for 11 hours (final pressure drop is 182 cm. of mercury). Final filtration efficiency is 88%, and averaged overall efficiency is about 80%. After 6% of the total time, particulate residue in the effluent is less than 2 parts per million.

#### EXAMPLE VI

Using a 4.84 cm. diameter polyethylene batt and apparatus as shown in FIGURE 6, three more wood-flour impregnated strands are made using differing concentrations both of the 300-mesh wood flour and of the added binder.

The binder employed is a high molecular weight, hot water-soluble polyvinyl alcohol which, in 4% solution at 20° C., exhibits a viscosity by the Hoeppler falling ball method of between 55 and 65 centipoises. Strand withdrawal rate for each case is 15.3 meters/min.

In each of the three cases, the suspension comprises 2 liters of water, 20 cc. of isoctyl phenyl polyethoxy ethanol, X cc. of a 10% aqueous solution of the polyvinyl alcohol, and Y gm. of the wood flour.

| Case No. | X  | Y   |
|----------|----|-----|
| 1-----   | 15 | 75  |
| 2-----   | 20 | 100 |
| 3-----   | 40 | 100 |

Even for the third case, involving relatively high binder concentration, the dried impregnated strand retains the flexibility characteristic of known impregnated tow products. Properties are shown in Table IV.

TABLE IV.—PROPERTIES OF THREE WOOD-FLOUR/POLY-ETHYLENE STRANDS

| Case No. | Denier | Twist<br>(turns/cm.) | Breaking<br>Strength<br>(kg.) | Residual<br>Elongation<br>Percent |
|----------|--------|----------------------|-------------------------------|-----------------------------------|
| 1-----   | 2,532  | 0.40                 | 1.52                          | 36.3                              |
| 2-----   | 3,197  | 0.31                 | 1.28                          | 37.1                              |
| 3-----   | 3,465  | 0.37                 | 1.40                          | 29.4                              |

#### EXAMPLE VII

An impregnated strand comprising cut nylon flock and plexifilamentary linear polyethylene is described.

The suspension is formed from 1 gram of cut nylon flock and one liter of water containing 1% of isoctyl phenyl polyethoxy ethanol. The flock is prepared by cutting 3 to 5 denier nylon filament into random lengths between 0.5 and 2 mm., the predominant length being about 0.75 mm.

A 4.84 cm. diameter polyethylene batt is immersed in the suspension as shown in FIGURE 1. Successive lengths are prepared by manually withdrawing about 1 meter of strand, adding twist of about 0.5 turns/cm., and cold stretching by about 10%. After several samples are withdrawn, examination of subsequent samples with a 5-power magnifying glass shows preferential longitudinal alignment of the flock within the composite strand.

#### EXAMPLE VIII

10 Fabric of asbestos impregnated yarn according to this invention is compared with an analogous fabric containing conventional asbestos yarn.

The anthophyllite asbestos shorts selected are known 15 to have excellent resistance to acid, alkali, and heat but to exhibit poor spinnability and poor flexibility. Dry screen analysis (U.S. Sieve Series) shows 46% of the shorts to be less than 65-mesh and 0% larger than 6-mesh.

A suspension is prepared from 500 gm. of asbestos 20 shorts, 8 liters of water containing 1% of isoctyl phenyl polyethoxy ethanol, and 75 cc. of the sodium silicate solution of Example II. A 4.84 cm. diameter polyethylene batt of about 800 denier plexifilament is impregnated according to FIGURE 6, strand withdrawal rate being 38 25 meters/min. and rotation of batt-holder 16 being at 1000 r.p.m. The dried impregnated strand contains between 10 and 15% polyethylene and weighs from 4.6 to 5.4 gm./10 meters. This strand corresponds to an 8 to 10 cut commercial yarn.

30 A plain-weave fabric from the strand of this example has 4.54 warp and 6.30 fill yarns/cm., weighs about 382 gm./m.<sup>2</sup>, and is 1.42 mm. thick. The fabric is soft and smooth and possesses unusually soft conformability. To the contrary, an analogous fabric woven from 10-cut 35 commercial asbestos yarn as fill shows the usual fuzziness and is so stiff that it cannot drape or conform readily.

35 Pressed for 15 minutes under 315 kg./cm.<sup>2</sup> pressure between platens heated to 155° C., the fabric of this example becomes stiff and looks wet. Subsequent unrestrained heating for 2 minutes in a 200° C. oven causes no shrinkage, and the cooled product shows good strength retention.

#### EXAMPLE IX

45 Impregnated strands comprising the diatomaceous earth of Example V and linear polyethylene plexifilaments are prepared according to a statistical design of variables and used to construct minifilters. The operating conditions which vary are shown in Columns 2-5 of Table V. In 50 each case a 4.84 cm. diameter polyethylene batt is impregnated according to FIGURE 6 at a constant wind-up rate for the product of 7.65 m./min. Each suspension is composed of the weight of diatomaceous earth shown in Column 2, the volume of emulsion binder shown in

55 Column 3, and 2 liters of water containing 1% of isoctyl phenyl polyethoxy ethanol. The binder emulsion contains 45±0.5% of a polyvinyl chloride copolymer of 0.1 to 0.2 micron particle size. The batt is rotated at the rate shown in Column 4, and the stretch indicated in Column 5 is imposed on the impregnated strand. Each dried product is transferred from its collection reel onto a conventional textile 30° paper cone, and the percentage loss in weight by dusting of diatomaceous earth during this step is given in Column 6.

60 Minifilters are constructed from each strand. They are formed on 1.91 cm. diameter, 17.15 cm. long perforated tubes, each perforation being 3.18 mm. in diameter and triangularly spaced from others on 6.35 mm. centers. Each end of each tube is masked with vinyl tape to leave 65 perforations exposed along 9.53 cm. of length, and the tube is wound with 52 helical traverses along its central 14.6 cm. of length. The weight of the strand used, in gm./10 meters, is shown in Column 7; and filter porosity as pressure drop in cm. of water for air-flow at 14 liters/75 min. is given in Column 8.

TABLE V

| Sample No. | Diatomaceous Earth, gms. | Emulsion Binder, cc. | Rotation, r.p.m. | Imposed Stretch, percent | Weight Loss in corning, percent | Strand Weight, gms./10 m. | Mini-Filter Porosity cm. H <sub>2</sub> O for 14 liters air/min. |
|------------|--------------------------|----------------------|------------------|--------------------------|---------------------------------|---------------------------|------------------------------------------------------------------|
| 20-1       | 350                      | 21                   | 580              | 20                       | 2.8                             | 8.9                       | 6.6                                                              |
| 2          | 385                      | 23                   | 580              | 20                       | 1.7                             | 11.3                      | 5.3                                                              |
| 3          | 350                      | 42                   | 580              | 20                       | 3.65                            | 10.1                      | 7.6                                                              |
| 4          | 385                      | 46                   | 580              | 20                       | 4.3                             | 9.9                       | 7.1                                                              |
| 5          | 350                      | 21                   | 640              | 20                       | 2.7                             | 9.8                       | 4.3                                                              |
| 6          | 385                      | 23                   | 640              | 20                       | 11.9                            | 11.9                      | 8.2                                                              |
| 7          | 350                      | 42                   | 640              | 20                       | 3.7                             | 9.1                       | 3.6                                                              |
| 8          | 385                      | 46                   | 640              | 20                       | 3.2                             | 9.5                       | 2.5                                                              |
| 21-1       | 350                      | 21                   | 580              | 9                        | 0                               | 8.4                       | 7.0                                                              |
| 2          | 385                      | 23                   | 580              | 9                        | 0                               | 11.2                      | 6.1                                                              |
| 3          | 350                      | 42                   | 580              | 9                        | 0                               | 8.1                       | 5.3                                                              |
| 4          | 385                      | 46                   | 580              | 9                        | .51                             | 8.8                       | 5.6                                                              |
| 5          | 350                      | 21                   | 640              | 9                        | 0                               | 8.4                       | 3.1                                                              |
| 6          | 385                      | 23                   | 640              | 9                        | .84                             | 9.9                       | 6.4                                                              |
| 7          | 350                      | 42                   | 640              | 9                        | 0                               | 9.5                       | 4.9                                                              |
| 8          | 385                      | 46                   | 640              | 9                        | 0                               | 9.3                       | 3.1                                                              |

Examination of these results shows that the dusting loss of Column 6 decreases markedly at lower levels of imposed stretch. Pressure drop for constant air-flow also decreases (i.e., porosity increases) with decreasing imposed stretch. For lower twist levels, porosity decreases at higher levels of binder; but the reverse is true at the high levels of twist. Dusting loss increases for increased twist at low levels of binder, but is insensitive to twist at high binder levels. The amount of impregnation by the diatomaceous earth is primarily a function of its concentration in the slurry, particularly at lower levels of binder. Decreased imposed stretch decreases the amount of impregnation.

#### EXAMPLE X

Wood-flour impregnated strands are prepared using linear polyethylene plexifilamentary batts of varying sizes and shapes. Processing is according to FIGURE 1 except that the suspension is continuously replenished, the fresh suspension composed of 200 gm. of wood flour, 5 liters of water, and 20 cc. of the isoctyl phenyl polyethoxy ethanol wetting agent. Table VI contains pertinent batt shapes and sizes as well as weights for the unimpregnated and impregnated plexifilaments.

TABLE VI.—BATTS OF DIFFERING SIZES AND SHAPES

| Batt Shape  | Dimensions (cm.) | End- Flexifila- ment, Denier | Plexifila- ment Weight (gm./10 m.) | Impregnated Strand Weight (gm./10 m.) |
|-------------|------------------|------------------------------|------------------------------------|---------------------------------------|
| Rectangular | 2.7 x 2.35       | 479                          | 0.43                               | 10.8                                  |
| Do          | 4.4 x 5.5        | 666                          | 0.60                               | 12.1                                  |
| Cylindrical | 2.35             | 180                          | 0.16                               | 3.9                                   |
| Do          | 4.84             | 967                          | 0.87                               | 27.5                                  |
| Do          | 10.80            | 1,178                        | 1.06                               | 22.0                                  |

The 4.84 cm. diameter batt is unexplainably more efficient than the others, but an almost linear relationship between impregnated strand weight and relaxed denier of the plexifilament exists for the other four.

#### EXAMPLE XI

Impregnation of plexifilamentary polyethylene with lead is described. A suspension of minus-300 mesh (U.S. Sieve Series) lead powder is prepared from 378 gm. of lead and 100 cc. of a 1% solution of non-ionic wetting agent in water. A 2 cm. long piece of 4.84 cm. diameter polyethylene batt is immersed in the suspension as shown in FIGURE 1, and the suspension is continuously agitated in its 250 ml. beaker using a rotary magnetic stirrer. An approximately 50 cm. long length of impregnated strand is manually withdrawn.

An exceedingly high pick-up of lead is attained. The wet strand weighs 1100 gm./10 meters, decreasing to 990 gm./10 meters on drying. The weight of dry strand is 1135 times greater than that of unimpregnated plexifilament, and the dry strand contains less than 0.1% linear polyethylene by weight.

20 The impregnated strand is also unusually cohesive and is, in fact, a soft rod about 6.5 mm. in diameter. A section of this product is fed to the nip between two solid metal 5.1 cm. diameter rolls rotating at about 20 r.p.m. The product emerging is a ribbon of plexifilament-reinforced lead about 12.7 cm. wide and from 0.28 to 0.46 mm. thick. The plexifilament apparently assists in drawing the strand into the nip of the rolls.

#### EXAMPLE XII

30 A suspension is prepared from 50 gm. of aluminum flake, 2 liters of water containing 20 cc. of isoctyl phenyl polyethoxy ethanol, and 10 cc. of the binder emulsion of Example IX. The aluminum flake is chemically pure aluminum of the type added as pigment to paint.

35 Operating in accordance with FIGURE 6, a 4.84 cm. diameter polyethylene batt is mounted in holder 16 and is rotated at from 320 to 345 r.p.m. Wind-up of impregnated strand is at 7.65 meters/min., Sample A receiving 9 to 10% imposed stretch, and sample B 40%.

40 An electrical charge decay test at 21.1° C. and 65% relative humidity (Rothchild charge decay) is performed by clamping specimens across the 2.54 cm. gap between to conductive clamps, imposing a voltage, and measuring the decay of imposed charge as a function of time. Sample A, weighing 1.25 gm./10 meters, decays as follows: 45 31.8% in 0.5 min.; 52.7% in 1.0 min.; 74.9% in 2 min.; and 100% in 10 min. Sample B, weighing 2.8 gm./10 meters, decays much more rapidly: 99.2% in 0.5 min.; 99.8% in 1 min.; and 100% in 2 min. Both samples are conductive for static electricity. An unimpregnated plexifilamentary polyethylene strand shows essentially no charge decay over extended periods of time. The composite strands of this example can be incorporated in minor amounts in fabrics of conventional yarn to prevent static build-up.

#### EXAMPLE XIII

50 A 0.3 gm. spongy mass of acicular boron nitride is suspended in 300 cc. of water by high-speed mixing. Volume of the suspension is then doubled by addition of a 1% aqueous solution of non-ionic wetting agent. A 4.84 cm. diameter polyethylene batt is treated as shown in FIGURE 6 except that no replenishment of suspension is provided. A twist of about 1 turn/cm. is applied, strand is withdrawn at 2 to 3 m./min., and 26% stretch is imposed before drying.

55 The weight gain by impregnation is so low that it cannot be computed by measuring the weight of impregnated strand. By dissolving the polyethylene in perchloroethylene, the initial product is shown to contain 3.96% solids, and a later product 1.29%.

60 Opaqueness of the plexifilamentary strand makes direct observation of longitudinal orientation of the acicular particles substantially impossible. One technique for detecting alignment is to press the impregnated strand to a

film between heated platens and then to examine the film at 250-diameter magnification under a circroscope. Definite longitudinal orientation of agglomerates of boron nitride particles is observed. It is observed that strands impregnated with boron nitride exhibit much less shrinkage and distortion on being pressed to a film than do unimpregnated plexifilaments. Stereocan photomicrographs of the uncompressed strands at magnifications up to 3000 also reveal agglomerates of boron nitride needles with a definitely preferred orientation along the strand axis. The strands can be used in place of conventional boron nitride strands as fillers in plastics.

#### EXAMPLE XIV

Using the procedure of Example XII, with an activated charcoal suspension rather than lead particles, another impregnated strand is obtained. The suspension is prepared from 50 gm. of activated charcoal and one liter of water containing 1% each of non-ionic wetting agent and the polyvinyl alcohol of Example VII.

After the manually withdrawn strand dries in air, its weight is 41 gm./10 meters at a diameter of 6 to 7 mm. Only 2.1% of the weight of the impregnated strand is polyethylene. It is almost free of dusting and is readily wettable by water. A fabric is woven from the composite strand material of this example to provide a convenient form for use in fume-absorption applications. It results that the 1% isoctyl phenyl polyethoxy ethanol added to the suspension as non-ionic wetting agent deactivates the activated charcoal with respect to fume-absorption. Another fabric prepared identically except that 10% of butanol is used as substitute wetting agent performs excellently in fume-absorption applications.

#### EXAMPLE XV

This example described the preparation of sponge yarns according to the method of this invention. In each of three cases, a 4.84 cm. diameter polyethylene batt is mounted as shown in FIGURE 1 and a strand is manually withdrawn.

In the first case, the suspension contains 13.5% cellulose and is composed of 70 gm. of viscose, 340 gm. of finely divided Glauber's salt, 43 gm. of water, and a trace of pink pigment. After cellulose regeneration, removal of Glauber's salt, and drying, the resultant sponge yarn weighs about 7 gm./10 meters. Its water absorbency is 13.4-fold by weight, and under mild finger pressure it wrings out to only 31.2% of its weight. The cellulose sponge is uniformly reinforced by the plexifilamentary strand matrix.

In the second case, the suspension is composed of 70 gm. of viscose, 340 gm. of finely divided Glauber's salt, 100 gm. of water, 0.2 gm. of isoctyl phenyl polyethoxy ethanol wetting agent, and a trace of pink pigment. Presence of wetting agent in this case increases the cross-sectional area of the impregnated strand by 6 to 8 times.

The third sample is prepared as in the second case except that the impregnated strand is sized by being drawn through the stem of a laboratory funnel to decrease its cross-sectional area to substantially that obtained in the first case.

The sponge yarns of this example can be used to make sponge mops. The yarns are superior to sponge yarns presently used for this purpose since the sponge is reinforced throughout its three dimensions by the plexifilamentary strand.

While these examples illustrated a great breadth of application of this process of preparing impregnated strands based on the plexifilamentary batts disclosed in Belgian Patents No. 670,293, they by no means exhaust the possibilities.

As an example, permanent magnets are produced from

crystalline particles of barium, lead, and strontium ferrites which, as disclosed in U.S. Patent No. 3,113,927, are exposed to a magnetic field before being sintered. Similar results can be expected from practice of this invention if the suspension is exposed to a magnetic field during strand-impregnation.

It is well-known to prepare yarns or fibers of intractable materials such as polytetrafluoroethylene or graphite using auxiliary carrier materials. The normally weak yarns are subsequently rendered coherent by, for example, fusion, sintering, or pyrolysis. Similar structures can be prepared using plexifilaments from batts as carriers.

In still another application, plexifilamentary strands are impregnated with diminutive seeds, such as tobacco or petunia seeds, to facilitate their handling and even distribution. They can simultaneously be impregnated with chemical agents, such as fungicides and fertilizers, to promote germination. Many other applications for metering particulate solids are immediately evident.

Still further, impregnated strands comprising drying agents, such as alumina and silica gel, or ion-exchange resins can be converted to fabrics for constructing belts or loops which can be mechanically and continuously moved through a unit where their function is employed and through a second unit where their function is regenerated.

It is known to encapsulate fluids, such as perfumes, medications, and cleaning agents, in wax, gelatin, or other microscopic hollow spheres. These fluids become active by rupture of their spheres in use. The impregnation of plexifilamentary strands with such "dry" fluids provides a convenient way to dispense and use them.

Finally, plexifilaments impregnated with a fibrous base and/or lubricants can serve excellently as packing materials in pumps, valves, and the like.

#### EXAMPLE XVI

A completely unexpected advantage of this invention is that the weight gains by impregnation as described herein are far greater than attained by any known method. This example provides comparison data in support of this observation. Table VII lists the pertinent data. In all cases, impregnation is accomplished as indicated in FIGURE 1. Two loose cotton rovings (one weighing 2.88 gm./10 meters with 1 turn per 2.54 cm., and the other weighing 3.00 gm./10 meters with 4 turns per 2.54 cm.) are compared with the use of a 4.84 cm. diameter linear polyethylene batt from which a plexifilamentary strand weighing only 0.86 gm./10 meters can be pulled. In Table VII, pairs of cotton-roving results are shown, the result at lower twist above that for higher twist. In each case, the suspension has the concentration of particulate material given in Columns 1 and 2. The dispersing medium is water containing about 1% of the isoctyl phenyl polyethoxy ethanol wetting agent.

From examination of Columns 3 and 4 it is immediately obvious that the low-weight plexifilament picks up far more particulate material than does the cotton roving. Columns 5 and 6 present the ratio of weights of dry impregnated strand and of unimpregnated base strand. For the plexifilament, these ratios are seen to be at least an order of magnitude higher than for cotton roving. In every instance, moreover, the cotton roving is found to be more coated than impregnated, while the plexifilamentary material is found to be uniformly impregnated throughout.

Over most of the concentration range for particulate material, the weight gain by impregnation increases substantially linearly with concentration, but, as is evident from Table VII, the highest concentrations are proportionately less efficient. This indicates the existence of a limiting concentration for practical and economical impregnation above which the suspensions become too viscous to penetrate the strands sufficiently rapidly. It is

apparent that the highest concentrations listed in Table VII are near the limiting concentrations.

TABLE VII.—COMPARISON IMPREGNATION OF COTTON ROVINGS AND POLYETHYLENE PLEXIFILAMENT

| Particulate Material    | Concen-<br>tration<br>(gm./<br>100 cc.) | Dry Strand<br>Weight (gm./10<br>meters) |                    | Pickup Ratio<br>(Dry Weight/<br>Initial Strand<br>Weight) |                    |
|-------------------------|-----------------------------------------|-----------------------------------------|--------------------|-----------------------------------------------------------|--------------------|
|                         |                                         | Cotton<br>rovings                       | Plexi-<br>filament | Cotton<br>rovings                                         | Plexi-<br>filament |
| Diatomaceous Earth..... | 5                                       | 5.55                                    | 20                 | 1.95                                                      | 23.3               |
|                         |                                         | 4.08                                    |                    | 1.38                                                      |                    |
|                         | 10                                      | 8.85                                    | 39                 | 3.14                                                      | 45.3               |
|                         |                                         | 6.60                                    |                    | 2.20                                                      |                    |
|                         | 20                                      | 10.9                                    | 180                | 3.86                                                      | 209                |
|                         |                                         | 12.3                                    |                    | 4.11                                                      |                    |
| Wood Flour.....         | *25                                     | 9.2                                     | 180                | 3.24                                                      | 209                |
|                         |                                         | 8.7                                     |                    | 2.93                                                      |                    |
|                         | 2.5                                     | 4.00                                    | 30                 | 1.43                                                      | 34.9               |
|                         |                                         | 4.36                                    |                    | 1.47                                                      |                    |
|                         | 5                                       | 6.80                                    | 59                 | 2.40                                                      | 68.6               |
|                         |                                         | 5.40                                    |                    | 1.82                                                      |                    |
| .....                   | 7.5                                     | 7.62                                    | 99                 | 2.68                                                      | 115                |
|                         |                                         | 6.55                                    |                    | 2.20                                                      |                    |
|                         | *10                                     | 7.95                                    | 118                | 2.78                                                      | 137                |
|                         |                                         | 9.20                                    |                    | 3.14                                                      |                    |

\*Near maximum concentrations.

Furthermore, impregnation of plexifilaments according to this invention has a completely unexpected concentrating effect with respect to the dispersed particulate materials. This is evidenced in three separate observations.

First, with increasing concentration of particulate material in the suspension, the ratio of wet to dried weight of impregnated strand decreases, i.e., the wet strand retains a noticeably higher relative proportion of solids. Thus, the wet/dry weight ratios for the strands of Table VII are, in order: 6, 4.5, 3.1, and 2.5 for diatomaceous earth; and 5.35, 5.35, 5.0, and 4.5 for wood flour.

Secondly, regardless of particle concentration, the weight of dry strand computed from the weight of wet strand and from the known suspension-concentration is always less than the measured dry weight. This indicates that the particles are preferentially removed from the suspension, a fact which could be applied, for instance, to the removal of solid wastes from effluent streams. For example, with reference to Table VII for the suspension containing diatomaceous earth at 5 gm./100 cc., the wet weight of the strand produced is 118 gm./10 meters. Subtracting the 0.86 gm./10 meters weight of plexifilament yields a weight pick-up of 117.14 gm./10 meters which, if it has the same particle concentration as the suspension (4.76 gm. of solid per 100 gm. of suspension), should contribute 5.58 gm. of dry particles to the 10-meter strand. The measured dry weight is, however, 20.0 minus 0.86 gm./10 meters, indicating that 3.43 times as much impregnation by solid particles is attained over the amount expected. Similar calculations for the 2.5 and 5.0 gm./100 cc. concentrations of wood flour yield ratios of 7.50 and 3.83 respectively.

Lastly, as shown in several examples, the concentration of particulate material in suspensions unreplenished by fresh suspension decreases with continued impregnation, which also shows preferential removal of the particles.

As illustrated in the examples, the ratio of the weight of particulate material to the plexifilamentary material in the composite strand can vary widely, depending upon the specific gravity of the particulate material, its concentration in the suspension, the size and shape of the particles, etc. Thus, the weight of the particulate material may be as little as 0.01 times the weight of the plexus or even less, or it may be as great as 1500 times the weight of the plexus or even greater. As indicated previously a particular advantage of the process of this invention is that the weight gains are far greater than attained by known impregnation methods. Thus it is in preparing composite yarns wherein the weight of the particulate material is several fold (e.g., 5 to 1000 fold) the weight of the

plexifilamentary material that the process offers its most significant advantage.

It is not completely understood why the process of this invention is so unexpectedly efficient in impregnating the plexifilamentary strand with particulate solids. At least a portion of the explanation seems, however, to depend on the cone (3 in the figures) of plexifilamentary plexus which forms as strand is drawn from a batt. Thus, as a tiny volume of plexifilament at the end of a batt is pulled out into an open plexus, it suddenly generates a much greater new volume which, when the cone is at least partially immersed in suspension, creates a pumping effect moving suspension into the strand. The results indicate the existence of at least two processes. First, suspension in large volume is pumped into the expanded plexus. Secondly, while the plexus collapses, a portion of suspension must be squeezed back out with selective filtration of particles by the condensing plexifilament. Thus, there is enhanced accumulation of particles within the strand. This concentration by filtration is apparently more efficient for lower suspension concentrations. Whatever the explanation, it is clear that impregnation according to this invention is different in kind from and superior to known impregnation and coating operations.

A pair of companion impregnations tends to confirm both the pumping and the filtration effects of the collapsing plexus. Two portions of a 4.84 cm. diameter polyethylene batt are separately impregnated while completely immersed (as in FIGURE 1) in a 3% suspension of asbestos shorts. One portion is first bored out to provide a 0.5 inch (1.27 cm.) diameter hole axially along its whole length. The hollow portion picks up about 54 gm. of asbestos per 1000 inches (25.4 meters) of strand-length while the solid portion picks up only about 41 gm. This is consistent with the hypotheses that a pumping effect draws fresh suspension through the hollow center and that the concentration of suspension reaching the center is greater than results if the suspension is all filtered in through the plexus of fibrils in the cone.

Numerous uses for this invention are disclosed in the foregoing examples and specifications. Many other uses and applications of the invention will be readily apparent to those skilled in the art.

I claim:

1. A process for making a composite strand comprising solid particulate material uniformly distributed throughout a three-dimensional integral plexus of synthetic organic polymeric film-fibril elements which comprises:
  - (a) providing a suspension of solid, particulate material in a dispersing medium;
  - (b) mounting a rod-shaped batt of longitudinally collapsed continuous plexifilamentary strand material such that a cone of plexifilamentary strand material pulled from one end of said batt is at least partially immersed in said suspension; and
  - (c) continuously pulling said plexifilamentary strand from said batt through said suspension.
2. A process as defined in claim 1 wherein said rod-shaped batt is continuously rotated to impart twist to the strand.
3. A process as defined in claim 1 wherein said cone is substantially completely immersed in said suspension.
4. A process as defined in claim 1 wherein stretch-elongation is imparted to said strand after impregnation by said suspension.
5. A process as defined in claim 1 wherein said suspension is continuously replenished to maintain a substantially constant concentration of particulate material.
6. A process as defined in claim 1 wherein said rod-shaped batt is axially bored.
7. A process as defined in claim 1 wherein said suspension includes a binder.

15

## References Cited

## UNITED STATES PATENTS

|           |        |                  |              |
|-----------|--------|------------------|--------------|
| 3,181,225 | 5/1965 | Knoepfler et al. | 28—75        |
| 3,193,407 | 7/1965 | Keller et al.    |              |
| 3,244,545 | 4/1966 | Marzocchi et al. | 28—75 XR     |
| 3,317,335 | 5/1967 | Marrinan et al.  | 117—138.8 XR |
| 3,321,903 | 5/1967 | Tawzer           | 57—153 XR    |
| 3,328,198 | 6/1967 | Koller           | 117—140 XR   |

16

|           |         |                |           |
|-----------|---------|----------------|-----------|
| 3,354,013 | 11/1967 | Terrell et al. | 156—152   |
| 3,365,346 | 1/1968  | Fritz et al.   | 156—152   |
| 3,382,662 | 5/1968  | Seelig et al.  | 57—149 XR |

DONALD E. WATKINS, Primary Examiner

U.S. CL. X.R.